

## UNITED STATES PATENT OFFICE

2,058,873

## ELECTRIC CURRENT CARRYING ELEMENT

Franz R. Hensel, Indianapolis, Ind., assignor, by  
mesne assignments, to P. E. Mallory & Co. Inc.,  
Indianapolis, Ind., a corporation of Delaware

No Drawing. Application June 25, 1935,  
Serial No. 28,303

5 Claims. (Cl. 219—4)

This invention relates to electrical contacting elements and the like such as welding electrodes and electrical contacts generally.

The present application comprises a continuation in part of my copending application, Serial Number 6,857, filed February 16, 1935.

An object of the invention is to improve the strength, hardness and temperature-resistant properties of contacting elements of the type disclosed.

Another object is to improve the electrical characteristics of such elements, including their conductivity and arc-snuffing properties.

Further objects are to prevent oxidation of the contacting elements both during and after formation thereof.

A specific object is to produce contacting elements, such as welding electrodes, contacts, trolley shoes and wheels, and contactors generally.

Other objects of the invention will be apparent from the following description taken in connection with the appended claims.

Alloys of copper and zinc in various proportions have been made and used commercially for many years. These alloys, in the cast form, are quite soft and can only be hardened to a very limited extent by cold working. Furthermore, the increased hardness can only be retained at fairly low temperatures. If these alloys are heated very substantially the hardness is lost and can only be regained by further cold working.

Copper-chromium alloys, on the other hand, while having many desirable properties, offer difficulties in casting and working, have a marked tendency to deteriorate through oxidation during and after casting and working, have a tendency to excessive grain growth during treatment and are quite susceptible to arcing when used for some electrical purposes, such as for welding electrodes.

The present invention comprises the combination of elements, methods of manufacture, and the product thereof brought out and exemplified in the disclosure hereinafter set forth, the scope of the invention being indicated in the appended claims.

While a preferred embodiment of the invention is described herein, it is contemplated that considerable variation may be made in the method of procedure and the combination of elements without departing from the spirit of the invention.

The invention contemplates the provision of a contacting element formed of an alloy of copper, chromium and zinc. This alloy, as will be apparent from the following description, possesses a

number of desired characteristics for such purposes not found in the binary alloys of copper and chromium or copper and zinc in addition to most of the desirable characteristics of these binary alloys.

The completed copper-chromium-zinc contacting element, to have the most desirable characteristics should contain the component ingredients in the following ranges of proportions:

|          |             |    |
|----------|-------------|----|
| Zinc     | 0.1 to 5.0% | 10 |
| Chromium | 0.1 to 2.5% |    |
| Copper   | Remainder   |    |

The preferred alloy for most contactors, including welding electrodes, has a composition, when completed, approximately as follows:

|          |           |    |
|----------|-----------|----|
| Zinc     | 0.5%      | 10 |
| Chromium | 0.5%      |    |
| Copper   | Remainder |    |

Another suitable alloy for contacting elements has the composition:

|          |           |    |
|----------|-----------|----|
| Zinc     | 0.75%     | 20 |
| Chromium | 1.50%     |    |
| Copper   | Remainder |    |

This alloy may sometimes be used as the final composition or it may be diluted with an equal proportion of copper resulting in a final alloy of the following approximate composition:

|          |           |    |
|----------|-----------|----|
| Zinc     | 0.3%      | 30 |
| Chromium | 0.5%      |    |
| Copper   | Remainder |    |

It will be noted that some of the zinc and chromium are lost in remelting due to oxidation and volatilization.

The casting qualities and the heat of recrystallization of the present alloy may be improved by the addition of silver in proportions above those normally found as an impurity in copper, and up to 5%. The cost, of course, will be increased thereby.

The zinc used in producing the present alloy is utilized in two ways. Part of it is used up as a deoxidizer and part of it remains as an ingredient in the finished alloy. In order to have 0.5% zinc in the finished alloy, for example, it is necessary to introduce 0.55% to 0.65% of zinc into the original melt. About half of the excess zinc is consumed as a deoxidizer, the zinc being converted to zinc oxide and separating as a slag. The rest of the excess is volatilized due to the low boiling point of the zinc. This volatilized zinc, when it comes into contact with the air, at a

high temperature forms zinc oxide which leaves the crucible in the form of a white smoke.

In the further treatment of the alloy after solidification it may be first heated to a temperature of 600° C. to 1050° C., and preferably above 700° C. for a short time, such as from 10 to 30 minutes. After the metal has reached the desired temperature it may be cooled quickly from the high temperature (quenched). The next step is preferably to heat treat the quenched alloy at a temperature of 350° C. to 600° C. for a period of from 10 minutes to 30 hours, depending on the temperature, the percentage of hardener used, and the results desired.

15 The alloy may then be cold worked to obtain a cold reduction of approximately 20% and further cold reduction, up to 50% or more, may be applied to further increase the hardness. It has been found that the conductivity will not be appreciably decreased by these further reductions.

20 For a maximum hardness and conductivity, however, it is preferable to apply a series of cold reductions alternated with relatively low temperature heat treatment, preferably within the range 400° C. to 500° C. The number of cold workings with intermediate heat treatments may vary with the properties desired in the finished product.

25 Instead of the cold working, the alloys may be hot forged according to usual methods and it will be found that the resulting hot-forged product will also have a hardness greater than the alloys of the prior art previously mentioned.

30 Alloys having the above mentioned proportions of zinc 0.3% and chromium 0.5% have been obtained after heat treatment with an electrical conductivity of 79.85% of that of pure forged copper and a Brinell hardness of 130. Such high conductivity in an alloy of such high hardness is very desirable for many of the applications mentioned and has been difficult to obtain in the past.

35 Another alloy containing 1.50% zinc, 0.60% chromium and the remainder copper, when cast and heat treated, has been obtained at a hardness of 65-70 on the Rockwell B scale and a conductivity of approximately 65% that of copper. After a cold reduction of about 25% the hardness was increased to 30 Rockwell B.

40 The heat-resistant properties of the present alloy are likewise greatly improved, the hardness and electrical conductivity being maintained indefinitely at temperatures in the order of 400° C. to 475° C.

45 Since the zinc acts as a strong deoxidizer it is not necessary to add other deoxidizers commonly used, such as silicon, aluminum or magnesium, for this purpose.

50 The presence of the zinc likewise tends to prevent excessive surface oxidation in the finished, solidified alloy and is particularly advantageous where they are heated to high temperatures. The surface oxidation in copper-chromium alloys is quite serious since the oxygen penetrates along the grain boundaries and tends to make 55 the alloy brittle. In the present alloy, the chromium is protected by the zinc, which will oxidize in preference to the chromium.

55 As is well known, zinc added to pure copper tends to decrease its conductivity quite considerably. It is surprising, therefore, to find that alloys of copper, chromium and zinc exhibit comparatively high electrical conductivity in the cast and heat treated state. With the addition of 0.5% or less of zinc the conductivity is not reduced below 75% to 80% and with even 1.5%

zinc the conductivity is found to be at least 65% that of copper when the alloy is in the cast, heat treated condition.

5 The alloy likewise has improved arc-snuffing properties, due to the presence of the zinc. This is highly advantageous for the electrical applications, such as in the use of the alloy for pressure welding electrodes and as a contact material. The low-boiling zinc (930° C.) tends to produce a gaseous phase which extinguishes the 10 arc. These arcing characteristics are improved by increasing the proportions of zinc.

15 This alloy is further characterized by small grain size. Copper-chromium materials must be heated to above 900° C. before quenching in water. That elevated temperature, however, is normally very conducive to grain growth, the size of the grains usually depending on the length of time the material is held at the elevated temperature. With the present alloy, containing zinc, the grain 20 size appears to be considerably reduced from that found in other copper-chromium alloys.

25 In the present alloy the proportions of zinc are kept below 5% and accordingly no low-melting point phase is formed, such as that formed in alloys containing zinc in high proportions. This allows a wider range of forging or hot working temperatures and presents a decided improvement over such alloys as copper-chromium-cadmium in which the forging range is very small. 30

35 The contacting element of the present invention is exceptionally well adapted, because of the above properties, to the production of resistance welding electrodes, contacts, trolley shoes, trolley wheels, contactors, electrical conductors, and the like. For each application the hardener may be used in such proportions as to obtain the desired hardness and conductivity.

40 While the present invention, as to its objects and advantages, has been described herein as carried out in specific embodiments thereof, it is not desired to be limited thereby but it is intended to cover the invention broadly within the spirit and scope of the appended claims.

45 What is claimed is:

1. A welding electrode composed of 0.1 to 5.0% zinc, 0.1 to 2.5% chromium and the remainder copper.

2. A welding electrode containing about 0.1 to 5.0% zinc, 0.1 to 2.5% chromium and the remainder substantially all copper, characterized by the combination of high hardness and high electrical conductivity.

3. An electric current carrying member containing about 0.1 to 5.0% zinc, 0.1 to 2.5% chromium and the remainder substantially all copper, characterized by a combination of high hardness and high electrical conductivity, and further characterized by the ability to maintain its hardness and high conductivity at temperatures in the order of 400° C.

4. An electric current carrying member containing about 0.1 to 0.75% zinc, 0.1 to 2.5% chromium and the remainder substantially all copper, characterized by a combination of high hardness and high electrical conductivity, and further characterized by the ability to maintain its hardness and high conductivity at temperatures in the order of 400° C.

5. An age-hardened electrical contact element 70 containing about 0.1 to 5.0% zinc, 0.1 to 2.5% chromium and the remainder substantially all copper, characterized by the combination of high hardness and high electrical conductivity.